

# United States Patent

[11] 3,607,394

|                                                                                                        |                                                                                                                                                                                                                  |                                                                                                                                                                                                                                                                                                                                                                                                                       |                       |  |
|--------------------------------------------------------------------------------------------------------|------------------------------------------------------------------------------------------------------------------------------------------------------------------------------------------------------------------|-----------------------------------------------------------------------------------------------------------------------------------------------------------------------------------------------------------------------------------------------------------------------------------------------------------------------------------------------------------------------------------------------------------------------|-----------------------|--|
| [72] Inventors                                                                                         | Felix Joseph Germino<br>12414 83 rd Ave., Palos Park, Ill. 60464;<br>Gerald Donald Miller, 3621 Douglas Road,<br>Downers Grove, Ill. 60515; Jerry Adam<br>Moskaluk, 14500 Sawyer Ave., Midlothian,<br>Ill. 60445 | [56]                                                                                                                                                                                                                                                                                                                                                                                                                  | References Cited      |  |
|                                                                                                        |                                                                                                                                                                                                                  | UNITED STATES PATENTS                                                                                                                                                                                                                                                                                                                                                                                                 |                       |  |
| [21] Appl. No.                                                                                         | 829,083                                                                                                                                                                                                          | 1,901,109                                                                                                                                                                                                                                                                                                                                                                                                             | 3/1933 Maier .....    |  |
| [22] Filed                                                                                             | May 29, 1969                                                                                                                                                                                                     | 2,314,459                                                                                                                                                                                                                                                                                                                                                                                                             | 3/1943 Salzburg ..... |  |
| [45] Patented                                                                                          | Sept. 21, 1971                                                                                                                                                                                                   | 2,900,335                                                                                                                                                                                                                                                                                                                                                                                                             | 8/1959 Bravos .....   |  |
|                                                                                                        |                                                                                                                                                                                                                  | 3,137,592                                                                                                                                                                                                                                                                                                                                                                                                             | 6/1964 Protzman ..... |  |
|                                                                                                        |                                                                                                                                                                                                                  | 3,434,880                                                                                                                                                                                                                                                                                                                                                                                                             | 3/1969 Kircher .....  |  |
| OTHER REFERENCES                                                                                       |                                                                                                                                                                                                                  |                                                                                                                                                                                                                                                                                                                                                                                                                       |                       |  |
| Ward Pigman, ed., "The Carbohydrates," 676, Academic Press, New York, 1957.                            |                                                                                                                                                                                                                  |                                                                                                                                                                                                                                                                                                                                                                                                                       |                       |  |
| Primary Examiner—Morris O. Wolk                                                                        |                                                                                                                                                                                                                  |                                                                                                                                                                                                                                                                                                                                                                                                                       |                       |  |
| Assistant Examiner—Sidney Marantz                                                                      |                                                                                                                                                                                                                  |                                                                                                                                                                                                                                                                                                                                                                                                                       |                       |  |
| Attorneys—Frank E. Robbins, Janet E. Price, Robert D. Weist, Martha A. Michaels and Dorothy R. Thumler |                                                                                                                                                                                                                  |                                                                                                                                                                                                                                                                                                                                                                                                                       |                       |  |
| [54] NOVEL PREGELATINIZED STARCHES AND<br>PROCESS FOR PREPARING SAME                                   | 5 Claims, No Drawings                                                                                                                                                                                            | <b>ABSTRACT:</b>                                                                                                                                                                                                                                                                                                                                                                                                      |                       |  |
| [52] U.S. Cl.....                                                                                      | 127/32,<br>75/2, 127/69                                                                                                                                                                                          | Pregelatinized starches are prepared by pasting an aqueous slurry of a starch which contains at least 50 percent amylopectin at a temperature of at least 300° F, and then rapidly, preferably instantaneously, removing the water therefrom as by roll or spray drying. The resultant products rapidly disperse in water to form smooth pastes which are characterized by low initial viscosity and minimal setback. |                       |  |
| [51] Int. Cl.....                                                                                      | C13I 1/08                                                                                                                                                                                                        |                                                                                                                                                                                                                                                                                                                                                                                                                       |                       |  |
| [50] Field of Search.....                                                                              | 127/28, 32,<br>69, 70, 71                                                                                                                                                                                        |                                                                                                                                                                                                                                                                                                                                                                                                                       |                       |  |

## NOVEL PREGELATINIZED STARCHES AND PROCESS FOR PREPARING SAME

This invention relates to cold water dispersible starch products and to a method for preparing same.

So-called "pregelatinized" starches, i.e. starches which have been gelatinized and dried and which will disperse when added to cold water to form pastes, have long been known to the art. They are generally prepared either by first gelatinizing an aqueous slurry of starch, as by heating it to its gelatinization temperature, and then instantaneously removing the moisture, as by means of a roll or spray drier, or, alternatively, by passing an aqueous slurry of granular (i.e. ungelatinized) starch through a suitable apparatus, e.g. a roll or spray drier, wherein the starch is simultaneously gelatinized and dried.

When an ordinary (i.e. unmodified and underivatized) starch is subjected to a conventional "pregelatinizing" treatment the product will, upon addition to cold (i.e. room temperature) water, form a smooth, relatively viscous paste. For certain applications, pregelatinized starches which will form pastes of low viscosity are desirable; such products are customarily prepared by hydrolyzing the starch, as with acid or enzyme, prior to or simultaneously with the pregelatinizing treatment. Hydrolysis causes molecular degradation of the starch, that is to say, it breaks down the starch molecules; because of this the resultant pastes are not only low in viscosity but low in molecular weight as well.

Another feature of pastes prepared from ordinary pregelatinized starch is their tendency to increase in viscosity upon standing; this characteristic is generally referred to as "setback." Conventionally, setback is minimized by derivatizing the starch, i.e. adding substituent groups to the molecule.

We have discovered a simple, rapid, and inexpensive method for preparing pregelatinized starches having the ability to disperse rapidly in cold water to form exceptionally smooth pastes, which pastes are characterized by low initial viscosity and exceptionally good viscosity stability (i.e. minimal setback). Furthermore, unlike conventional pregelatinized starches which have been subjected to hydrolysis to lower their paste viscosity, the starches of our invention are characterized by substantially no, or at most very slight, molecular degradation.

It is an object of the present invention to prepare cold water dispersible starches which will reconstitute to form pastes having low initial viscosity and minimal setback.

Another object is to prepare pregelatinized starches which will rapidly disperse in cold or warm water to form exceptionally smooth pastes of low viscosity.

An additional object is to treat starch in such a way that the molecules of same will be substantially undegraded, but pastes of the starch will nevertheless exhibit low viscosity and exceptionally good viscosity stability.

Other objects and advantages will be apparent from the specification and the appended claims.

Briefly, the process is as follows. A granular starch which contains at least 50 percent amylopectin is slurried in water and pasted at a temperature of at least about 300° F., after which the water is instantaneously removed.

The starch can be any starch provided it contains at least about 50 percent amylopectin. Cereal starches, such as those derived from corn, wheat, barley, etc.; tuber starches, such as those obtained from potatoes, tapioca, or the like; and the "waxy starches," e.g. waxy maize, waxy rice, and waxy sorghum, which consist entirely or substantially entirely of amylopectin, and are all suitable for the practice of the invention. The "high amylose" starches, i.e. those which contain 60 percent amylose or more, as well as amylose itself, are not suitable, in that these starches produce products which form gels upon reconstitution with water, and gel formation is an undesirable characteristic in the applications for which the products of the invention find their greatest utility. The starches can be modified and/or derivatized prior to the pasting treatment. The only critical requirements for starches to be treated in accordance with the invention are (1) they must be granular, i.e. ungelatinized, (2) they must be capable of being gelatinized in water (for example, a starch which is so

highly cross-linked that it will not undergo gelatinization could not be used), and (3) they must contain at least 50 percent amylopectin.

The instantaneous removal of the water after the high temperature pasting can be performed in any suitable apparatus, e.g. a drum drier, a spray drier, a belt drier, a foam mat drier, or the like, the only requirement being that the apparatus be capable of drying the starch paste very rapidly.

The original slurry can contain up to about 35 percent starch solids (by weight, based on the weight of the total slurry). As stated before, the starch must be pasted at a temperature of at least about 300° F. The only upper temperature limit is that at which substantial molecular degradation of the starch will take place, e.g. over about 450° F. Temperatures of from about 315° F. to about 360° F. are preferred.

It is very important that the paste not be permitted to cool to a point at which the starch begins to retrograde or becomes aggregated prior to removal of the water. The temperature at which retrogradation or aggregation begins depends upon the solids content of the paste. For example, a 35 percent solids paste will begin to retrograde at about 190° F., while one of 12 percent solids will begin to retrograde at about 140°-150° F. Also, it is preferred that the paste be fed to the drier very quickly after the completion of the pasting step, because the longer it is held at a high temperature the greater is the likelihood of molecular degradation and/or crystallization.

The products, because of their ability to reconstitute in cold water to form smooth pastes of relatively low viscosity, high molecular weight and minimal setback, are extremely useful as adhesives and as coatings and sizings for paper and textiles. It has also been observed that the reconstituted pastes have excellent film-forming properties, i.e., they will readily form films which exhibit excellent oil holdout and water holdout properties. The products are also excellent iron oxide depressants in the calcium soap flotation process for concentrating iron ores.

Structurally, the products of the invention are characterized by complete granular fragmentation, as contrasted with the conventional pregelatinized starches which contain a certain amount, usually about 10-15 percent, of intact granules.

The following examples will illustrate the practice of the invention. They are intended for illustrative purposes only, and should not be construed as limiting the scope of the invention in any way.

### EXAMPLE I

A series of runs was made in which aqueous slurries, at 25 percent solids concentration by weight, of regular, unmodified corn starch were heated in a steam injection cooker to temperatures of from 212° F. to 355° F. until they were completely pasted. Immediately after pasting the products were passed over a 24 inch roll drier, operated at 2.6 r.p.m. and 100 lbs. steam, the skin temperature of the rolls being 284° F. The dried products were removed from the rolls by means of doctor blades and permitted to cool. Pastes of the products were prepared by adding the starch in various concentrations to warm water, with stirring. Viscosities of the pastes were then determined with a Brookfield viscometer at 20 r.p.m. Two samples were held for 24 hours at 150° F., after which their viscosities were again measured.

The pasting temperatures, concentrations of the reconstituted pastes and viscosities of the reconstituted pastes are given in Table I.

TABLE I

| Pasting temp., ° F. | Concentration of reconstituted pastes, weight percent | Brookfield viscosity of reconstituted pastes at 150° F., cps. | Brookfield viscosity of reconstituted pastes after 24 hours at 150° F., cps. |
|---------------------|-------------------------------------------------------|---------------------------------------------------------------|------------------------------------------------------------------------------|
| 212                 | 20                                                    | *600,000                                                      | -----                                                                        |
| 250                 | 20                                                    | 300,000                                                       | -----                                                                        |
| 300                 | 20                                                    | 55,000                                                        | -----                                                                        |
| 355                 | 30                                                    | 24,000                                                        | 35,000                                                                       |
| 355                 | 10                                                    | 1,200                                                         | 1,800                                                                        |

\*Approximately.

As can be seen from Table I, pastes of starches prepared in accordance with the invention (cooked at temperatures of 300° F. and 355° F.) were substantially lower than those cooked at 212° F. and 250° F.

As can also be seen from the table, pastes of starches prepared in accordance with the invention which were held for 24 hours increased only slightly in viscosity.

Blender at 4,000 r.p.m. prior to addition to the pulp. In run 5 the alkaline starch dispersion was cooked at 100° C. for 15 minutes prior to addition to the pulp.

Table II sets forth the amounts of starch used in each run (calculated on the basis of pounds of starch per ton of ore), and the analyses of the froth and concentrate portions of each run.

TABLE II

| Run No. | Corn starch used                | Lb. starch per ton ore | Product           | Percent weight | Percent Fe     | Percent Fe recovery |
|---------|---------------------------------|------------------------|-------------------|----------------|----------------|---------------------|
| 1.....  | Prepared according to invention | 3                      | Froth Concentrate | 25.94<br>74.06 | 33.65<br>62.21 | 15.93<br>84.07      |
| 2.....  | Regular                         | 3                      | Froth Concentrate | 51.00<br>49.00 | 47.75<br>62.71 | 44.21<br>55.79      |
| 3.....  | Regular                         | 4                      | Froth Concentrate | 23.90<br>76.10 | 30.40<br>62.64 | 13.23<br>86.77      |
| 4.....  | Homogenized regular             | 3                      | Froth Concentrate | 21.70<br>78.30 | 28.19<br>62.31 | 11.24<br>88.76      |
| 5.....  | Cooked regular                  | 3                      | Froth Concentrate | 48.72<br>51.28 | 46.73<br>62.88 | 41.39<br>58.61      |

## EXAMPLE II

An aqueous slurry at 25 percent solids of white milo starch was pasted at 335° F. in a steam injection cooker and immediately roll dried as in Example I. The product was added to warm (175° F.) water with stirring at a concentration of 26 percent solids; the starch readily dispersed to form a smooth paste. The Brookfield viscosity (at 20 r.p.m.) was 7,200 c.p.s.

## EXAMPLE III

A 16 percent aqueous slurry of regular unmodified corn starch was pasted at 360° F. in a Votator indirect heat exchanger. Immediately after pasting the product was dried in a spray drier. A 25 percent solids paste was prepared in water at 110° F. The Brookfield viscosity of the paste was 126,000 c.p.s.

The example was repeated using wheat starch, waxy rice starch and potato starch with comparable results. In all cases the products rapidly dispersed in water to form smooth pastes which were characterized by low initial viscosity and minimal setback.

## EXAMPLE IV

This example illustrates the use of starch prepared in accordance with the invention in the concentration of iron ores.

The standard laboratory procedure for ore flotation, a description of which follows, was employed.

A 500-gram sample of iron ore is pulped to 30 percent solids in a batch laboratory conditioner. To this is added a 2 percent starch dispersion prepared by stirring the starch in 0.5 N sodium hydroxide solution for 30 minutes at room temperature. The pH of the pulp and starch mixture is adjusted to 11.8 and the pulp is conditioned for 2 minutes. This is followed by 1-minute conditioning with calcium chloride (2 lbs. per ton ore) and then 2 minutes conditioning with Actinol FA-2 (0.8 lb. per ton). The conditioned pulp is transferred to a Fagergren laboratory flotation machine, diluted to 20 percent solids, and floated for 5 minutes. The froth and the concentrate are then weighed and analyzed for iron content.

Five runs were made, employing different starches as follows. Run 01 used a corn starch treated in accordance with Example I, pasted at 340° F. Runs 2 and 3 employed regular, unmodified corn starch in two different amounts. In run 4 regular unmodified corn starch was used, and the alkaline starch dispersion was homogenized for 5 minutes in a Waring

From the percent iron recovery in the concentrates, it is evident that at 3 lbs. starch per ton of ore the starch of the invention is more effective than regular starch and than regular starch that has been cooked. It is nearly as effective as starch that has been subjected to extensive shearing in a blender or as regular starch used at the increased rate of 4 lbs. per ton. Advantages in the use of starch prepared in accordance with the invention are that less of it needs to be used as a depressant and that its dispersions do not need to be sheared extensively to be obtained in a useful form.

While the invention has been described in connection with specific embodiments thereof, it will be understood that it is capable of further modification, and this application is intended to cover any variations, uses, or adaptations of the invention following, in general, the principles of the invention and including such departures from the present disclosure as come within known or customary practice in the art to which the invention pertains and as may be applied to the essential features hereinbefore set forth, and as fall within the scope of the invention.

What is claimed is:

1. Process for preparing a pregelatinized, cold water dispersible starch product comprising:
  1. heating an aqueous slurry of a granular starch, said granular starch containing at least 50 percent amylopectin, at a temperature of at least about 300° F. for a time sufficient to paste completely said starch, and
  2. thereafter rapidly removing substantially all of the moisture from the pasted starch.
2. Process of claim 1 wherein the moisture is removed by roll-drying the pasted starch.
3. Process of claim 1 wherein the moisture is removed by spray drying the pasted starch.
4. Process of claim 1 wherein said starch slurry is heated at a temperature within the range of between about 315° F. and about 360° F.
5. A pregelatinized starch product which will rapidly disperse in water to form a smooth paste having low initial viscosity and excellent viscosity stability, said starch being further characterized by complete granular fragmentation and substantially no molecular degradation, said starch having been prepared in accordance with the process of claim 1.